

## UNITED STATES PATENT OFFICE

2,440,954

PROCESS FOR ELIMINATING STAIN FROM  
COLOR-YIELDING ELEMENTS BY TREAT-  
MENT WITH AROMATIC ALDEHYDES CON-  
TAINING AN ACYL GROUPAndrew Bradshaw Jennings, New Brunswick,  
N. J., assignor to E. I. du Pont de Nemours &  
Company, Wilmington, Del., a corporation of  
DelawareNo Drawing. Application August 23, 1945,  
Serial No. 612,300

6 Claims. (Cl. 95—88)

1

This invention relates to color photography and more particularly to the elimination of color stain from colloid layers of photographic elements. Still more particularly it relates to a process and compositions for eliminating stain from photographic colloid silver halide layers of color yielding elements.

The most commercially practical methods of color photography at the present time utilize the principle of color coupling development of developable silver salt images. This principle has been known for many years and is described in Fischer United States Patent 1,102,028. Color formers are utilized in such processes which couple with the development reaction products of aromatic primary amino photographic developing agents to produce quinoneimine or azomethine dyes. This action takes place during the reduction of silver salts to metallic silver, the dyes being formed in situ with metallic silver images. The color formers can be used either in water-permeable colloid-silver halide layers or in aqueous developer solutions. Many variations and improvements on the process described in the Fischer patent have been proposed. In one of such processes the color formers are of relatively high molecular weight or are polymeric in nature and are incorporated in gelatino-silver halide emulsion layers. Because of their molecular size and chemical constitution, they do not migrate during photographic processing. In another variation the color formers are placed in gelatin layers which are contiguous with gelatino-silver halide emulsion layers. A recent and novel process is described in United States Patent 2,397,864. In this process hydroxylated polymer color formers are used as binding agents for silver salts. These color formers have the dual function of producing color during color development and of being binding agents for the silver salts. They may be distinguished from gelatin and gelatin color formers in that they do not set and do not form gels.

A disadvantage which is common to all of the above processes is that a color fog or stain is formed during processing to form quinoneimine or azomethine dye images. When the exposed photographic silver halide layers are developed with a primary aromatic amino developing agent a dye fog is frequently formed in the emulsion

2

layers. This is so because the developing agents suffer oxidation to some extent by the action of air and the oxidized developer tends to couple with the color former at points or areas in the colloid layers of the photographic elements where no silver image is produced. In addition, in processing films of the above type it is frequently observed that there is a pronounced tendency for the generation of the color in the non-image areas of the colloid layers in the color yielding photographic elements when the color developed element is treated with an oxidizing bleach solution used for the purpose of removing metallic silver and silver salts from the layers. This undesirable aspect results from a retention of small amounts of development reaction products of the aromatic primary amino developing agents in the colloid layers following color coupling development. It is difficult, if not impossible, to remove the last traces of such reaction products by washing the film in aqueous baths.

An object of this invention is to provide a simple and economical method of eliminating color stain from color-yielding photographic elements. Another object is to provide such a method which is applicable to all types of photographic elements utilizing color formers in the formation of quinoneimine or azomethine dye images. Still other objects will be apparent from the following description of the invention.

The above disadvantages of the prior art process of color coupling development are overcome and the above objects are obtained by treating photographic silver halide emulsion layers containing quinoneimine or azomethine dye images with a ketaldone containing in addition to the amine-active group, that is, the carbonyl group of the aldehyde or ketone, a solubilizing group. Suitable solubilizing groups which may be present in the ketaldones include carboxyl, primary amide, amino, hydroxyl, sulfonic acid, and primary sulfonamide groups. The photographic elements containing such emulsion layers can be treated during the development of the metallic silver and quinoneimine or azomethine dye images or after development has been completed. Thus the ketaldones containing the solubilizing groups are present at the time of formation of the silver images or subsequently thereto but prior to the bleaching steps.

The ketaldones apparently combine chemically with the primary aromatic amino developing agents and/or with the development reaction products of such agents formed during the reduction of the silver salt images and form products which have a markedly greater solubility than the developing agents or their development reaction products themselves. The solubilized products can readily be removed from the colloid layers of the elements by a simple washing step.

The invention will be further illustrated but is not intended to be limited by the following examples.

*Example I*

A photographic film element was prepared by depositing on a cellulose acetate film base a gelatin dispersion containing comminuted silver and the mixed acetal of salicylaldehyde and benzaldehyde ortho sulfonic acid with polyvinyl acetal. A red-sensitive green blind gelatino-silver halide emulsion was then coated on the layer formed. Next was coated a gelatin dispersion of 4,4'-o-sulfo-benzylidene-bis-(1-phenyl-3-methyl-5-pyrazolone) to form a color-yielding layer. Next was coated a green-sensitive gelatino-silver iodobromide emulsion. On the resulting layer was then coated a gelatin dispersion of yellow colloidal silver and 4,4'-o-sulfo-benzylidene-bis-(1-phenyl-3-methyl-5-pyrazolone). On the layer formed was coated a gelatin dispersion containing benzoylacetylureoylacetsenizide. On the resulting color-yielding layer was then coated a blue-sensitive gelatino-silver iodobromide emulsion. Three strips of the resulting film element were exposed to a multi-colored object and then developed in a solution of the following composition:

|                                  | Grams |
|----------------------------------|-------|
| N-methyl-p-aminophenol.½ sulfate | 5.0   |
| Hydroquinone                     | 7.5   |
| Sodium sulfite (anhydrous)       | 60.0  |
| Potassium bromide                | 4.5   |
| Water to 1000 cc.                |       |

to form silver images and washed and dried. The elements were then reexposed to white light and color developed in a solution of the following composition:

|                                  | Grams |
|----------------------------------|-------|
| N-diethyl-p-phenylenediamine.HCl | 2.5   |
| Sodium carbonate                 | 40.0  |
| Potassium bromide                | 5.0   |
| Water to 1 liter.                |       |

One strip was washed for a period of 20 minutes which was required to insure the absence of a pinkish stain caused by oxidation of traces of developer left in the film and it was then bleached in a 4% potassium ferricyanide solution and fixed in a 25% hypo solution whereby a multicolor image was formed. The image was somewhat clouded by the presence of a light pinkish stain. The other two strips were bathed immediately after color development in a 5% aqueous solution of benzaldehyde ortho sulfonic acid sodium salt and then washed for 5 and 10 minutes respectively before bleaching and fixing in similar baths. The strip which had been washed for 5 minutes had a trace of a pinkish stain but the strip which had been treated for 10 minutes was free from stain.

*Example II*

A cellulose nitrate film base was coated with a gelatin dispersion of comminuted silver. On the

resulting layer there was coated a gelatin dispersion of 4,4'-bis-(1-naphthol-2-sulfoamidophenyl) ether. On the layer which formed was then coated a red-sensitive green blind gelatino-silver iodobromide emulsion layer. On the emulsion layer was coated a gelatin dispersion containing 4,4'-bis-(1-naphthol-2-sulfoamidophenyl) ether. On the layer which formed was then coated a gelatin dispersion of 4,4'-o-sulfobenzylidene-bis-(1-phenyl-3-methyl-5-pyrazolone). On the resulting color-yielding layer was then deposited a green-sensitive gelatino-silver iodobromide emulsion layer. Next was coated a gelatin dispersion containing colloidal silver and 4,4'-o-sulfobenzylidene-bis-(1-phenyl-3-methyl-5-pyrazolone). Next was coated a gelatin dispersion containing benzoylacetylureoylacetsenizide. On the resulting color-yielding layer was then coated a blue-sensitive gelatino-silver iodobromide emulsion. The resulting multilayer film was exposed to a color scene and then developed in a developer solution prepared by admixing the following components:

|                                     | Grams |
|-------------------------------------|-------|
| 25 N-methyl-p-aminophenol.½ sulfate | 2.0   |
| Hydroquinone                        | 9.0   |
| Sodium sulfite (anhydrous)          | 60.0  |
| Sodium carbonate (anhydrous)        | 40.0  |
| Potassium hydroxide                 | 3.5   |
| 30 Potassium thiocyanate            | 2.0   |
| Water to 1000 cc.                   |       |

The film was washed for 20 minutes in running water and dried. After exposure to white light the film was developed for 25 minutes in a solution of the following composition:

|                                      | Grams |
|--------------------------------------|-------|
| p-Aminodiethyl aniline hydrochloride | 2.5   |
| Potassium carbonate                  | 25.0  |
| Potassium thiocyanate                | 2.5   |
| 40 Benzaldehyde-o-sulfonic acid      | 5.0   |
| Water to 1000 cc.                    |       |

The benzaldehyde-ortho-sulfonic acid used in the developer solution had no deleterious effect upon the developer action. It was found to be very effective in reducing the amount of stain. Concentrations ranging from .5 to 5.0 grams per liter were tried with good results. An increased amount of the compound shortened the time of washing. The samples in which the benzaldehyde-ortho-sulfonic acid had been added to the developer showed a markedly less tendency to produce stain than a control sample in which no sulfonic acid had been added to the developer.

*Example III*

A multilayer film of the type disclosed in Example II was treated in an aqueous solution containing 2% of benzaldehyde-o-sulfonic acid after the first and non-color forming development had been completed. It was found that the ortho-sulfonic acid could be used in a concentration of 1-10% with good results. The film is immersed for a period of 2-10 minutes and is substantially free from color stain after photographic processing to a multicolor image has been completed.

*Example IV*

A mixture of 100 parts of polyvinyl alcohol having a viscosity of 18-28 centipoises in a 4% aqueous solution at 20° C., 200 parts of salicylaldehyde, 500 parts of dioxan, and 10 parts of 85% phosphoric acid is stirred at 85° C. for 5 hours, diluted with 1000 parts of acetone and filtered. The white powder is washed by decantation in 1000-part

portions of acetone 6 times for 1 hour each, then filtered and dried to give 140 parts of a fine white powder. Ten parts of this powder is dissolved by stirring in 90 parts of 40% ethanol-water at 80° C. for one-half hour. To 40 parts of this solution is added 40 parts of water, 5 parts of 1% aqueous sodium dodecyl sulfate, and 5 parts of concentrated ammonia water. The mixture is stirred at 45° C. while adding 20 parts of 3N silver nitrate and 23 parts of 3N ammonium bromide- $\text{^{16}N}$  potassium iodide simultaneously during the five minutes. After stirring a total of 15 minutes, the silver halide dispersion is allowed to cool and mixed with 100 parts of acetone which precipitates the binding agent containing dispersed light-sensitive silver halides. After pouring off the liquid, the soft rubbery polymer mass is washed for one-half hour in running water to remove the soluble salts, then the remaining 60 parts of the original polymer solution is added, together with 10 parts of ethanol and 1 part of 10% aqueous potassium bromide, and the whole mixture stirred at 58% C. for one-half hour, after which it may be used directly or stored. This light-sensitive dispersion is coated on paper or a film base and exposed to a colored object. It is then developed in the following solution:

|                                     | Grams |
|-------------------------------------|-------|
| p-Aminodiethylaniline hydrochloride | 4.0   |
| Potassium carbonate                 | 60.0  |
| Potassium bromide                   | 3.5   |
| Sodium sulfite (anhydrous)          | 20.0  |
| Benzaldehyde-o-sulfonic acid        | 5.0   |
| Water to 1000 cc.                   |       |

The film after washing and bleaching in Farmer's reducer was found to be free from any significant color stain.

In place of using the ketaldone containing solubilizing groups in the developing baths or washing baths they may be treated following normal color development in a stop bath or an acid fixing bath. Baths such as the following may be employed:

*Stop bath #1*

|                              | Grams |
|------------------------------|-------|
| Sodium sulfite               | 15    |
| Benzaldehyde-o-sulfonic acid | 5     |
| Water to 1000 cc.            |       |

*Stop bath #2*

|                              | grams | cc |
|------------------------------|-------|----|
| Sodium acetate               | 50    |    |
| Acetic acid                  |       | 5  |
| Benzaldehyde-o-sulfonic acid | 5     |    |
| Water to 1000 cc.            |       |    |

*Stop bath #3*

|                              | Grams |
|------------------------------|-------|
| Sodium busulfite             | 30    |
| Benzaldehyde-o-sulfonic acid | 5     |
| Water to 1000 cc.            |       |

*Fixing bath*

|                              |       |     |
|------------------------------|-------|-----|
| Sodium thiosulfate           | grams | 240 |
| Sodium sulfite               | do    | 6   |
| Boric acid                   | do    | 6   |
| Acetic acid (28%)            | cc    | 35  |
| Potassium alum               | grams | 12  |
| Benzaldehyde-o-sulfonic acid | do    | 5   |
| Water to 1000 cc.            |       |     |

In place of the benzaldehyde ortho sulfonic acid and its sodium salt which are described in the above examples, there may be substituted various other ketaldones which contain solubilizing groups and are amine-active. Suitable additional compounds of this type include benzaldehyde-p-sulfonic acid, benzaldehyde-m-sulfonic acid, phthalaldehydic acid, hydroxybenzalde-

hyde, glyoxylic acid, alpha-naphthaldehyde-beta-sulfonic acid, 2-naphthaldehyde-3-sulfonic acid, 1-naphthaldehyde-4-carboxylic acid, 2-naphthaldehyde-3-carboxylic acid, pyruvic acid, levulinic acid and their alkali metal and ammonium salts, the amide of phthalaldehydic acid, and benzaldehyde-o-sulfonamide.

The present process is not limited to the use of the particular photographic elements described above. On the contrary, it may be used with any multilayer or single layer or films having light-sensitive silver halide layers which utilize color formers in the chromogenic development of the silver salts. Thus the photographic elements described in United States Patents 2,319,369, 2,319,426, 2,320,422, 2,328,034, 2,282,001, 2,363,764, and various other patents may be similarly treated.

An advantage of the present invention is that it considerably reduces the time of aqueous processing of photographic elements. To be more specific, it reduces the time of washing to eliminate color stain to a marked degree.

A further advantage of the invention is that it provides a simple and economical means for eliminating color stain from photographic films utilizing chromogenic development. The elimination of all traces of such stain is highly important to the faithful reproduction of highlight tones in a color photograph. Another advantage of the invention is that it may be used with all types of photographic film elements which utilize color formers which form quinone-imine or azomethine dyes during color coupling development.

As a result of the fact that the effective solubility of the color-coupling developers is increased, contact with the skin is less harmful since washing results in complete removal. This is highly important since many aromatic amines of this type are capable of producing certain varieties of dermatitis.

As many widely different embodiments of this invention can be made without departing from the spirit and scope thereof, it is to be understood that the invention is not to be limited except as defined by the claims.

I claim:

1. The process which comprises treating a photographic element bearing at least one water-permeable layer containing a color developed dye image taken from the group consisting of quinoneimine or azomethine dye images and silver and silver salts with an aqueous solution containing a compound taken from the group consisting of unsubstituted benzaldehyde and naphthaldehyde monocarboxylic and monosulfonic acids and their alkali metal and ammonium salts.
2. The process which comprises treating a photographic element bearing at least one water-permeable layer containing a color developed dye image taken from the group consisting of quinoneimine or azomethine dye images and silver and silver salts with an aqueous solution containing an unsubstituted naphthaldehyde sulfonic acid.
3. The process which comprises treating a photographic element bearing at least one water-permeable layer containing a color developed dye image taken from the group consisting of quinoneimine and azomethine dye images and silver and silver salts with an aqueous solution containing an unsubstituted benzaldehyde sulfonic acid.
4. The process which comprises color develop-

ing an exposed photographic element containing reducible silver halide images in the presence of a color former in a developer solution containing a primary aromatic amino color developing agent and a compound taken from the group consisting of unsubstituted benzaldehyde and naphthaldehyde monocarboxylic and monosulfonic acids and their alkali metal and ammonium salts.

5. The process which comprises color developing an exposed photographic element containing reducible silver halide images in the presence of a color former in a developer solution containing a primary aromatic amino color developing agent and an unsubstituted benzaldehyde monocarboxylic acid in an amount of 0.5 to 5.0 grams per liter of developer solution.

6. The process which comprises color developing an exposed photographic element containing reducible silver halide images in a water-permeable colloid layer, in the presence of a color former, in an aqueous alkaline developer solution containing a primary aromatic amino color developing agent and from 0.5 to 5.0 grams per liter of solution of benzaldehyde-*o*-sulfonic acid.

ANDREW BRADSHAW JENNINGS.

## REFERENCES CITED

The following references are of record in the file of this patent:

## UNITED STATES PATENTS

|    | Number    | Name               | Date           |
|----|-----------|--------------------|----------------|
|    | 2,154,895 | Fricke et al.      | Apr. 18, 1939  |
|    | 2,154,918 | Schneider et al.   | Apr. 18, 1939  |
| 10 | 2,169,513 | Brunken            | Aug. 15, 1939  |
|    | 2,286,662 | Weyde              | June 16, 1942  |
|    | 2,301,387 | Evans              | Nov. 10, 1942  |
|    | 2,322,027 | Jelley             | June 15, 1943  |
| 15 | 2,356,477 | Staud              | Aug. 22, 1944  |
|    | 2,356,486 | Weissberger et al. | Aug. 22, 1944  |
|    | 2,360,290 | Vittum et al.      | Oct. 10, 1944  |
|    | 2,367,548 | Vittum             | Jan. 16, 1945  |
|    | 2,378,265 | Vittum et al.      | June 12, 1945  |
| 20 | 2,384,658 | Vittum             | Sept. 11, 1945 |
|    | 2,384,663 | Weissberger et al. | Sept. 11, 1945 |

## FOREIGN PATENTS

|  | Number  | Country       | Date          |
|--|---------|---------------|---------------|
|  | 462,140 | Great Britain | Mar. 3, 1937  |
|  | 836,144 | France        | Oct. 10, 1938 |